

Jan. 3, 1950

C. W. MacCONNELL

2,493,461

MEANS AND METHOD OF FORMING PIEZOELECTRIC CRYSTALS

Filed May 4, 1944

2 Sheets-Sheet 1



*Fig. I*



*Fig. II*

INVENTOR.  
CHARLES W. MAC CONNELL  
BY  
*Louis L. Vagnon*  
ATTORNEY

Jan. 3, 1950

C. W. MacCONNELL

2,493,461

MEANS AND METHOD OF FORMING PIEZOELECTRIC CRYSTALS

Filed May 4, 1944

2 Sheets-Sheet 2



Fig. III



Fig. V



Fig. VI



Fig. VII

INVENTOR.  
CHARLES W. MacCONNELL

BY  
Louis A. Gagnon  
ATTORNEY

## UNITED STATES PATENT OFFICE

2,493,461

## MEANS AND METHOD OF FORMING PIEZO-ELECTRIC CRYSTALS

Charles W. MacConnell, Southbridge, Mass., assignor to Harvey-Wells Communications, Inc., Southbridge, Mass., a corporation of Massachusetts

Application May 4, 1944, Serial No. 534,137

6 Claims. (Cl. 171—327)

1

This invention relates to piezo-electric crystals and more particularly to efficient and economical means and method of processing said crystals whereby their resultant frequency and output characteristics may be more simply and positively controlled.

This application is a continuation in part of my copending application, Serial No. 423,017, filed December 15, 1941 and which has matured into Patent 2,353,171 issued on July 11, 1944.

One of the principal objects of the invention is to provide improved means and method of processing piezo-electric crystals whereby the said crystals may be made to oscillate properly and may be more positively and economically controlled as to frequency of oscillations and may be more permanently stabilized as to activity and as to said frequency of oscillations.

Another object is to provide more stable or aged piezo-electric crystals and method of making the same.

Another object is to provide improved means and method of lapping piezo-electric crystals whereby substantially parallel surfaces may be formed on the opposed sides of said crystals in a simple and efficient manner and of subsequently subjecting said crystals to acid etching for rendering said crystals more permanently stable as to activity and frequency control.

Another object is to provide novel means and method of economically processing precision crystals of given frequency values and of aging or stabilizing said crystals as to activity and frequency output.

Another object is to provide novel means and method of changing the frequency of a crystal which oscillates properly, but which is slightly off as to desired frequency, without materially altering its oscillating properties and for simultaneously rendering said crystal stable as to said desired frequency. Other objects and advantages of the invention will become apparent from the following description taken in connection with the accompanying drawings and it will be apparent that many changes may be made in the details of construction, arrangement of parts and steps of the method shown and described without departing from the spirit of the invention as expressed in the accompanying claims. It is therefore desired that the invention not be limited to the exact details of construction, arrangement of parts, and steps of the method shown and described as the preferred forms only have been given by way of illustration.

Referring to the drawings:

2

Fig. I is a perspective view of the device embodying the invention setting forth one step of the process of manufacture;

Fig. II is a sectional view taken as on line II—II of Fig. I and looking in the direction indicated by the arrows;

Fig. III is a sectional view taken as on line III—III of Fig. II looking in the direction indicated by the arrows and showing the sectional parts in full;

Fig. IV is a diagrammatic view illustrating a step of a modification in the method of the invention;

Fig. V is an exaggerated diagrammatic view of a crystal surface subsequent to the abrading of said surface;

Fig. VI is a view generally similar to Fig. V of said surface subsequent to controlled acid etching; and

Fig. VII is a greatly exaggerated diagrammatic view similar to Figures V and VI.

It has been usual in processing piezo-electric crystals to reduce the crystals to the proper size, working characteristics and frequency by very delicate hand controlled operations which depended entirely upon the skill of the operator.

One of the difficulties in processing piezo-electric crystals of the character described has been to obtain a substantially parallel relation of the side surfaces of the crystals while simultaneously reducing said crystals to the required uniform thickness. The uniform thickness is essential in obtaining the working characteristics or activity and frequency values desired of the crystals. Because of the necessity of exceptionally skilled labor in processing said crystals, in the past, and because of the delicate hand operations required to produce crystals of this nature, such crystals have been extremely difficult and costly to make. This was due to a great percentage of spoilage which inherently resulted from the hand controlled procedure of fabrication and is one of the many disadvantages which the present invention obviates.

Although the reducing of the crystals to uniform thickness by grinding or abrading has been found to be very practical from the viewpoint of saving time and cost, it has been found that crystals reduced to required frequency by this method possess surface irregularities and incipient fractures which during use or when stored for eventual use will break off and destroy the activity of the crystal.

The effect is similar to that of drawing a diamond across a piece of glass hardly leaving a

mark thereon but it is commonly known that pieces will fracture out or the fracture will extend entirely through the piece of glass causing cracks to occur.

It has also been found that if a crystal has gone bad on the shelf from incipient fractures, fine quartz powder will be found inside of the electrode holder if the crystal is put to use and forced to oscillate. Such fractures also alter the frequency of the crystal tending to cause the frequency of the crystal to increase due to the particles breaking off.

A major feature, therefore, of the present invention, in addition to reducing the surfaces of the crystals to parallelism by abrading, is to etch the crystals by dipping them in acid such as hydrofluoric acid or some other similar etching media to cause relatively pronounced protuberances, fractures and strains produced by the abrading operation to be etched sufficiently so as to prevent or avoid their breaking off or causing parts of the crystal to break off when stored or subsequently put to use. This removal of the fractures, etc. set forth above, causes the crystals to be more stable or produces a so-called aging of said crystals whereby their activity and frequency of oscillation will be more permanent and will not alter after a relatively long period of storage and when then put to actual use. This stabilizing also tends to increase the activity of the crystals and also permits a more positive frequency control to be obtained. This removal by etching is brought about simultaneously to the reducing of the crystal to the desired frequency of oscillation, the abrading being halted at a point which will permit removal of the material by etching to obtain the desired frequency and simultaneously stabilize the said frequency as to activity and frequency of oscillation by removing parts of the crystal which might have a tendency to break off through subsequent jarring, storing, or during actual use.

It is known in the art that crystals have been acid etched but such etching mainly has been for the purpose of initially exposing the twinning with said crystal being thereafter further etched to obtain the frequency desired.

It has been found by applicant that crystals etched to this extent are not desirable or practical for use. The etching according to applicant's findings on one hand must be sufficient to cause the bottoms of the fractures to become cupped or curved whereby the tendency for parts to break off is greatly reduced or eliminated and, on the other hand, must not be sufficient to cause a glazing or to cause the quartz structure to be too prominently brought out so that the structure is no longer substantially uniform. If the quartz crystals are etched too much, parts of the quartz will etch faster than others due to the crystalline structure, that is, parts of the crystalline body in certain orientation dissolves more rapidly than others and an undesirable structure will remain. The etching, therefore, must be carefully controlled so as to be sufficient to stabilize the crystals and simultaneously produce the frequency desired but not of an amount sufficient to cause too much of the more readily dissolvable portions of the crystal to be removed.

Referring more particularly to the drawings wherein like characters of reference designate like parts throughout the several views the device which performs one of the essential steps of the method, as shown in Figs. I through III, com-

prises broadly a lap 1 having a relatively flat surface 2 thereon. The said surface 2 has a plurality of communicating longitudinal grooves 3 therein which provide means into which excessive abrasive may flow from the effective surface of the lap. The piezo-electric crystal 4, which is to be lapped, is held in a holder 5 and is moved with said holder over the relatively flat surface 2 of the lap 1. The relation of the crystal with the holder and lap can best be seen in Fig. II. The holder 5 comprises a main upright portion 6 having a base 7 with a relatively flat surface 8 thereon. The main upright portion 6 has a longitudinal opening 9 extending throughout the major portion of the length thereof with a closed end 10 adjacent the base 7. The closed end has a reduced opening 11 therein communicating with the longitudinal opening 9. Internally of the opening 9 there is a pair of angularly disposed plates 12. The said plates 12 form a slideway for a slide plunger 13. The said slide plunger 13 is preferably of a triangular cross section and is held in desired frictional contact with the slide plates 12 by means of a pressure plate 14. The said pressure plate 14 is resiliently urged into engagement with the slide plunger 13 by pins 15 pressed toward the plate by backing springs 16. The said pins are slidably mounted within the threaded longitudinal bores 17 of spaced blocks 18. The blocks are attached to the upright 6 by suitable means such as pins or screws not shown. The tension of the respective backing springs 16 is varied by means of screws 19 threaded with the internally threaded bore of the blocks 18.

By adjustment of the screws 19 proper tension may be directed to the resilient backing springs 16, thereby setting up a pressure on the pins 15 suitable to retain the slide plunger 13 in different positions of adjustment longitudinally of the slide plates 12.

The slide plunger 13, adjacent the lower end thereof, is provided with a protruding portion 20 fitting within the opening 11. The protruding portion 20 has an end surface 21 which is substantially parallel with the surface 8 on the base and substantially perpendicular to the longitudinal axis of the slide plunger 13. The said slide plunger 13 has a knob-like member 22 adjacent the upper end thereof which is adapted to be engaged when it is desired to move the slide plunger 13 longitudinally of the slide plates 12. The size of the opening 11 and the contour thereof depends upon the size and shape of the crystal which is to be abraded and is preferably made slightly larger than the crystal.

The procedure of processing the crystal is substantially as follows: The crystal is first cut from the mother crystal in proper desired relation to the optical axis, electrical axis and one of the crystallization axes of the mother crystal, depending upon the characteristics desired of the completed crystal. A suitable abradant such as an ordinary mixture of emery and kerosene is placed on the surface 2 of the lap. The kerosene is preferably sprayed on the surface of the lap or applied thereto by an ordinary oil cup and the emery is in powder form and is shaken onto the surface of the lap. A second lap or means simulating the lap 1 is then placed on the surface of the lap with its effective abrading surface engaging the effective abrading surface of the lap 1 and is moved in a sidewise direction over said lap to work the abradant into the surface 2 of the lap 1 and to cause the excessive abrad-

ant to flow into the longitudinal grooves 3 of said lap. If there is an excessive amount of kerosene or abradant on the lap this may be blotted off through the use of suitable blotting paper or the like.

The crystal 4 is then placed in the opening 11 and is rested on the relatively flat end 21 of the portion 20. The said crystal is held in position while the holder 5 is slid onto the surface of the lap in a sidewise direction. After the said crystal and holder have been placed on the surface 2 of the lap 1 a pressure is exerted on the knob-like member 22 to cause the slide plunger 13 to move downwardly and urge the crystal 4 into engagement with the surface 2 of the lap. The tension resilient means 16 is such that the plate 14, functioning cooperatively with the slide plates 12, will frictionally hold the slide plunger 13 in adjusted position. The pressure is then released on the knob 22 and the holder 5 together with the crystal 4 is moved into a sidewise direction over the surface 2 of the lap 1. This causes the abradant on said surface 2 to remove a given amount from the engaging surface of the crystal. Because of the fact that the surface 21 on the end of the plunger 13 and the surface 8 on the base 7 are substantially parallel with each other, substantially equal pressure will be distributed throughout the area of the crystal and will cause the opposed surfaces thereof to be abraded substantially parallel with each other. Periodically during the abrading the crystal is removed and cleansed and is tested in a suitable testing device for determining its oscillating characteristics and frequency. If the crystal is of a slightly lower frequency than desired it is again placed in the holder 5 on the lap 1 and an additional amount is removed. By following this procedure the crystal may be reduced to the proper thickness to obtain the frequency and oscillating characteristics desired. The crystal, because of the particular arrangement of the holder 5 and lap 1, will more positively have its opposed surfaces formed in substantially parallel relation with each other and will therefore be of substantially constant thickness throughout, thereby insuring good working or oscillating characteristics. During the abrading the crystal is first abraded on one side for a given period of time and is then removed from the holder, cleansed, reversed, and again placed in the holder and abraded on the second side for a given period of time. This procedure more positively insures forming parallel surfaces on the crystal. During said periodic removal of the crystal from the holder it is tested to determine its frequency and also to determine its oscillating characteristics. The procedure is somewhat of a cut and try method.

The above procedure is followed to reduce the crystals to a desired predetermined thickness which preferably is not the final thickness required. The crystals are then preferably reduced in thickness by etching with a suitable acid, such as hydrofluoric acid. This may be accomplished by grasping the sides of the crystal by a suitable holder 23 and by dipping the crystal into a bath 24 of hydrofluoric acid for a given time interval, which is sufficient to obtain the desired frequency. After each dipping, the crystal is washed in water or other suitable liquid to remove the acid. This avoids the danger of altering the oscillating characteristics of the crystal and provides a means of obtaining the desired frequency without further abrading. It is to be understood that any known acid may be used.

In order for crystals to oscillate properly and at the desired frequency, the dimensional characteristics must be very carefully controlled. In following the teaching of the present invention, the crystals are preferably initially abraded to reduce the surface to substantially parallelism and to reduce the thickness to within controlled limits whereby a given required amount of the material of the crystal will thereafter have to be removed by acid etching in order to obtain the desired activity and frequency of oscillations. The amount allowed to remain on the crystal at the completion of the abrading is controlled so that it does not require undue etching. For example, the preferred amount to be removed must be sufficient to permit the stabilizing of the crystals and simultaneously avoid altering by glazing or altering the structure of the crystal body so as to bring out the quartz structure thereof too predominantly.

For example, the amount of material to be removed from the crystal is preferably determined by frequency change. The frequency change which is found to be most practical as produced by etching should be more than one-tenth percent of the frequency and less than one percent of the frequency of the crystal, the preferred amount being sufficient to bring about a frequency change of from about five-tenths percent to eight-tenths percent for any crystal. For example, for a crystal which is to have a frequency of 5000 kc., it is advisable to stop the grinding when the crystal has approximately 4970 kc. and to thereafter etch the crystal until it reaches 5000 kc. or preferably stop the grinding at 4980 kc. and stop the etching at 5000 kc. It is not advisable to grind to 4995 kc. and stop the etching at 5000 kc. because this would not be sufficient etching to stabilize the crystal. This same principle will apply to other frequencies. The etching is controlled preferably to remove the fractures due to grinding, that is, to cause the bottom of the fractures to become rounded whereby subsequent breaking off of parts of the crystal when stored or during actual use will be greatly reduced or obviated. The removal, however, should not be continued to a point where you get the development of the quartz crystal structure. There are strains around all fracture points in the quartz. The scratches or fractures resulting from grinding tend to spread similar to cracks in a piece of glass, particularly when the crystals are violently oscillated. The acid etching as referred to herein, therefore, is not only for the purpose of reducing the crystal to obtain accuracy as to its frequency of oscillation but must be of an amount sufficient to simultaneously remove fractures of the type which will progress upon use of the crystal or upon subsequent jarring or storage and must not be sufficient to bring out too predominantly the quartz crystal structure. As a result of acid etching to remove these fractures simultaneously to the obtaining of desired frequency of oscillation greater stability or aging is accomplished and more desirable working characteristics or activity is obtained. That is, crystals formed in this manner remained more permanently stable and can be stored for subsequent use over considerably long periods without loss of activity and with substantially no change as to frequency of oscillation and said crystals tend to maintain a more constant frequency of oscillation during use. The present method of etching quartz crystals does not in any way alter the working characteristics of the crystals but rather has a tendency to improve the activity. It is to be understood, of course, that it is

necessary to have the quartz for these crystals free from all types of twinning as is commonly known in the art and that several different cuts with respect to the orientation of the mother crystal may be formed as is commonly known. The present invention may be employed with any of the above cuts.

The word, activity, as set forth herein is intended to mean the starting ability of the crystal to oscillate or its ability to quickly respond to electrical exciting.

In Fig. V of the drawings, there is diagrammatically illustrated a crystal 26 having an abraded surface 27 thereon. It is particularly pointed out that the surface has an irregular formation resulting from the abrading operation when greatly magnified. The difficulty, as found in the past, is that such abraded surfaces have a plurality of fractures therein such as diagrammatically illustrated at 28. These fractures, when the crystals are stored or under conditions of use have a tendency, as illustrated by the dash-line 29 in Fig. V, to cause portions of the crystal to break away thereby altering the activity of the crystal and its frequency of oscillation. It is quite apparent that should a plurality of such pieces, as diagrammatically illustrated at 30, break away from the crystal the crystal would become greatly altered as to its frequency, and it has been found in the past, that the loss of activity is such as to render the crystals impractical for use.

In Fig. 6, the surface 27 is diagrammatically illustrated after having been acid etched. The fractured areas 28, are removed so as to produce curved bottom areas 31 and smoothened contour surface 32 whereby the tendency for parts, such as diagrammatically illustrated at 30, breaking off is greatly reduced or completely obviated.

Fig. 7 is a much greatly magnified view illustrating the features diagrammatically shown in Figs. 5 and 6. By etching the abraded surface thereof to remove the fractures as set forth above, a more stable or aged crystal is obtained. By aging, it is meant stability as to permanency of activity and frequency.

It is to be understood, of course, that when the crystals have been initially abraded that they are cleansed and checked as to their frequency subsequent to the final etching. This cleansing can be accomplished by a quick dip in the acid and a rinse in water to remove oil, grit, etc. from the crystal so that a fairly accurate check as to its frequency can be obtained prior to the final acid etching.

Although applicant has shown and described the abrading of only one surface of the quartz crystal at a time, it is to be understood that the said opposed surfaces of the crystal or crystals may be simultaneously abraded. This is accomplished by placing the crystals in a suitable holder between an upper and lower lap or abrading tools having flat surfaces in substantially parallel relation with each other and causing the crystals to be moved relative to the abrading surfaces of the laps or tools in the presence of a suitable abrasive such as oil, kerosene or other suitable liquid having powdered abrasive means therein such as emery, carborundum, crushed diamonds, etc.

In addition to moving the holder and crystals between abrading surfaces of the laps, one or both of the laps could be moved relative to each other while maintaining the abrading surfaces substantially parallel and while permitting one of the laps to move towards the other as the material is

removed from the crystals. In this manner a plurality of crystals may be reduced to desired thickness by abrading the opposed sides of the crystal simultaneously.

It is to be understood that the crystals are finished by acid etching as set forth above.

The acid used in etching may be of any desirable type which will attack the crystals such as hydrofluoric acid.

From the foregoing description, it will be seen that simple, efficient and economical means have been provided for accomplishing all of the objects and advantages of the invention.

Having described my invention, I claim:

1. A method of forming stabilized piezo-electric crystals comprising the steps of abrading to substantial parallelism the opposed surfaces of a crystal cut from the mother quartz to approximately required dimensions while simultaneously permitting the abrading action on said surfaces to introduce incipient fractures in the abraded surfaces of controlled depth, continuing the abrading action until the frequency value of the crystal has been increased to a value of from 0.1 to 1.0% lower than the final frequency required for the crystal, cleansing the surfaces of the crystal to remove remaining abrasive and loose particles of quartz and subsequently subjecting the cleansed crystal to an acid bath of a given concentration for an interval of time controlled according to the concentration of the bath sufficient to reduce said crystal to its required frequency, with said bath simultaneously rounding out the bottoms of said incipient fractures present in the abraded surfaces while avoiding the glazing of said surfaces of the crystal and the development of its crystalline structure.

2. A method of forming stabilized piezo-electric crystals comprising the steps of abrading the opposed surfaces of a crystal to substantial parallelism while subjected to a substantially uniform pressure throughout the area of said surfaces, said crystal having been cut from the mother quartz to approximately required dimensions and simultaneously permitting the abrading action of said surfaces to introduce incipient fractures in the abraded surfaces of controlled depth, continuing the abrading action until the frequency value of the crystal has been increased to a value of from 0.5 to 0.8% lower than the final frequency required for the crystal, cleansing the surfaces of the crystal to remove remaining abrasive and loose particles of quartz and subsequently subjecting the cleansed crystal to an acid bath of a given concentration for an interval of time controlled according to the concentration of the bath sufficient to reduce said crystal to its required frequency with said bath simultaneously rounding out the bottoms of said incipient fractures present in the abraded surfaces while avoiding the glazing of said surfaces of the crystal and the development of its crystalline structure.

3. In the method of forming stabilized piezo-electric crystals of quartz, the steps comprising subjecting the crystal to an acid bath of a given concentration, said crystal having opposed surfaces thereon abraded to substantial parallelism, with said surfaces containing incipient fractures of controlled depth resulting from the abrading action to which said surfaces have been subjected, and having been cleansed of abrasive and loose particles of quartz, said crystal having a frequency value of from 0.1 to 1.0% lower than the final frequency required for the crystal, and

causing said crystal to remain subjected to the acid bath for an interval of time controlled according to the concentration of the bath and sufficient to reduce said crystal to its required frequency, with said bath simultaneously rounding out the bottoms of said incipient fractures present in the abraded surfaces while avoiding the glazing of said surfaces of the crystal and the development of its crystalline structure.

4. In the method of forming stabilized piezoelectric crystals of quartz, the steps comprising subjecting the crystal to a chemical bath having characteristics for etching quartz and of a given concentration, said crystal having opposed surfaces thereon abraded to substantial parallelism, with said surfaces containing incipient fractures of controlled depth resulting from the abrading action to which said surfaces have been subjected, and having been cleansed of abrasive and loose particles of quartz, said crystal having a frequency value of from 0.5 to 0.8% lower than the final frequency required for the crystal, and causing said crystal to remain subjected to the acid bath for an interval of time controlled according to the concentration of the bath and sufficient to reduce said crystal to its required frequency, with said bath simultaneously rounding out the bottoms of said incipient fractures present in the abraded surfaces while avoiding the glazing of said surfaces of the crystal and the development of its crystalline structure.

5. The method of processing a piezo-electric crystal comprising placing the crystal within a recess in a holding member, said crystal having been initially cut from the mother quartz to approximately the required dimensions, placing said holding member and crystal on the abrading surface of a lapping tool, imparting a substantially uniform pressure on a side surface of said crystal throughout the area thereof while in said holder to cause the opposed surface of said crystal to engage the abrading surface of the lapping tool, moving said holder and crystal over the abrading surface of the lapping tool, and periodically reversing said crystal during said lapping so as to cause the opposed surfaces of the crystal to be reduced to substantial parallelism while permitting the abraded surfaces of the crystal to contain incipient fractures of controlled depth, continuing the lapping action on said surfaces until the frequency value of the crystal has been increased to a value of from 0.1 to 1.0% lower than the final frequency required for the crystal, cleansing the surfaces of the crystal to remove remaining abrasive and loose particles of quartz and subsequently subjecting the cleansed crystal to an acid bath of a given

concentration for an interval of time controlled according to the concentration of the bath and sufficient to reduce said crystal to its required frequency, with said bath simultaneously rounding out the bottoms of said incipient fractures present in the abraded surfaces while avoiding the glazing of said surfaces of the crystal and the development of its crystalline structure.

6. The method of processing a piezo-electric crystal comprising placing the crystal within a recess in a holding member, said crystal having been initially cut from the mother quartz to approximately the required dimensions, placing said holding member and crystal on the abrading surface of a lapping tool, said abrading surface having abrasive material uniformly distributed thereon, imparting a substantially uniform pressure on a side surface of said crystal throughout the area thereof while in said holder to cause the opposed surface of said crystal to engage the abrading surface of the lapping tool, moving said holder and crystal over the abrading surface of the lapping tool, and periodically reversing said crystal during said lapping so as to cause the opposed surfaces of the crystal to be reduced to substantial parallelism while permitting the abraded surfaces of the crystal to contain incipient fractures of controlled depth, continuing the lapping action on said surfaces until the frequency value of the crystal has been increased to a value of from 0.5 to 0.8% lower than the final frequency required for the crystal, cleansing the surfaces of the crystal to remove remaining abrasive and loose particles of quartz and subsequently subjecting the cleansed crystal to an acid bath of a given concentration for an interval of time controlled according to the concentration of the bath and sufficient to reduce said crystal to its required frequency, with said bath simultaneously rounding out the bottoms of said incipient fractures present in the abraded surfaces while avoiding the glazing of said surfaces of the crystal and the development of its crystalline structure.

CHARLES W. MacCONNELL.

#### REFERENCES CITED

The following references are of record in the file of this patent:

#### UNITED STATES PATENTS

| Number    | Name       | Date          |
|-----------|------------|---------------|
| 1,869,169 | Marrison   | July 26, 1932 |
| 2,323,569 | Hawk       | July 6, 1943  |
| 2,353,171 | MacConnell | July 11, 1944 |
| 2,364,501 | Wolfskill  | Dec. 5, 1944  |
| 2,376,219 | Winslow    | May 15, 1945  |
| 2,411,298 | Shore      | Nov. 19, 1946 |
| 2,417,179 | Ross       | Mar. 11, 1947 |